

No. 893,938.

PATENTED JULY 21, 1908.

J. F. MONNOT.

COMPOUND METAL BODY AND PROCESS OF PRODUCING SAME.

APPLICATION FILED APR. 13, 1907.



WITNESSES:

Gus. A. Klimek  
L. Hauerstein

INVENTOR

J. F. Monnot

Marble & Eddy  
ATTORNEYS

# UNITED STATES PATENT OFFICE.

JOHN F. MONNOT, OF NEW YORK, N. Y., ASSIGNOR TO DUPLEX METALS COMPANY, OF NEW YORK, N. Y., A CORPORATION OF NEW YORK.

## COMPOUND METAL BODY AND PROCESS OF PRODUCING SAME.

No. 893,933.

Specification of Letters Patent.

Patented July 21, 1908.

Application filed April 13, 1907. Serial No. 367,986.

*To all whom it may concern:*

Be it known that I, JOHN F. MONNOT, a citizen of the United States, residing at New York, in the county of New York and State 5 of New York, have invented certain new and useful Improvements in Compound Metal Bodies and Processes of Producing Same; and I do hereby declare the following to be a full, clear, and exact description of the same, 10 such as will enable others skilled in the art to which it appertains to make and use the same.

This invention relates to reinforced gold and processes of preparing the same and consists in metal articles composed of layers of 15 gold permanently united to backing layers of harder and stronger metals, and in particular to the ferrous metals, and also in a process of firmly and permanently uniting gold to such other metals by a union in the nature of 20 a weld union; all as more fully hereinafter set forth and as claimed.

Steel and the ferrous metals generally do not readily unite to the wholly unlike metal gold, either by cast-on unions or even by 25 electroplating, and gold and steel are seldom if ever directly united, despite the manifest advantages which such a combination of metals would offer. In electroplating, it is generally considered necessary to cover the 30 iron or steel with a preliminary coating of copper and then deposit the gold on the copper. Mercurial gilding, formerly frequently used, has now gone out of use because of its expense, dangerous nature and generally unsatisfactory results. The film produced, 35 while of course fitting snugly in all the surface irregularities of the steel and therefore adhering, has no real cohesion and readily strips, the stripping being much facilitated 40 by the fact that the coating is porous and permits permeation of moisture and corrosive gases to the underlying corrodible metal. Electrolytic coatings are also porous and readily strip, having no coherence with the 45 base metal. And in all these prior methods, it has been necessary to produce an article of the finished shape and then plate or otherwise coat with the gold, the coatings having no such union with the steel as would permit 50 coating an ingot or other intermediate article and subsequent coextending to form the finished article.

It is the object of the present invention to devise a method of producing unions between gold and steel, preferably autogenous 55

in character, which shall be firm, permanent and of the character of a weld, permitting indefinite coextension of the joined metals without separation and with preservation of the same relative thickness of such joined metals throughout the working, and producing metal articles of novel character.

I have discovered that the lack of affinity between steel and gold which subsists at all common temperatures and which renders 60 difficult their direct union by any of the known processes, though also existing at the common casting temperature of gold, disappears when the gold is raised to a temperature much above its melting point. When 65 steel is presented in a clean and non-oxidized condition to gold in this state which, for lack of another name, I have termed the "supermolten condition" the steel is readily wetted by the fluid gold and unites with it in some 70 manner not clearly understood, so that after solidification of the gold, the two metals 75 will be found autogenously and permanently united by a union in the nature of a weld-union, resisting rupture by cutting tools, flexure or sudden changes in temperature. For most mechanical purposes, the two joined metals will be found to be capable of 80 working as if one homogeneous piece of metal; as in drawing down, hammering, rolling, 85 and the like. This peculiar mutual affinity possessed by the high melting metals at temperatures much above their melting points, appears to be generic and in Patent No. 853,716, dated May 14th, 1907, I have 90 described and broadly claimed processes of uniting metals based on this fact.

Gold melts at about 1950° Fahrenheit and the supermolten temperature is about five hundred or more degrees above that temperature. Its alloys with copper, etc., such as coin gold, melt at much lower temperatures but a similar elevation of temperature above the melting point, whatever it may be, also brings them to a supermolten condition. 95 For the purposes of the present invention, either pure gold or its alloys may be employed. Gold so attached to steel, being put on in the fluid condition, shares in the peculiarity of fluids and set fluids in being 100 poreless, and as subsequent coextension of the joined metals further compacts the gold, obliterating blow-holes, cavities and the like, in the finished article the coating is absolutely impervious to fluids and gases, in this 105 110

respect being wholly unlike the usual fire-gildings and electroplatings.

In cases where it is deemed preferable to work with at least part of the gold at a less temperature, the same character of coating may be secured by the use of an expedient which consists in first filming the steel by contact with supermolten gold to form a superficial coating and then casting against the so-treated surface, gold at a more convenient casting temperature. Or the filmed surface may, though less advantageously, have solid or softened gold welded to it by mechanical force. Still another expedient is to substitute a film of copper in the initial treatment of the steel, dipping the steel into a bath of supermolten copper for this purpose. To this coppered surface ordinary coin gold, which contains copper, may be readily made to cohere by casting such gold against it.

In utilizing the described properties of supermolten gold, the steel to be coated may first be thoroughly cleaned, as by sandblasting and then heated under conditions precluding oxidation. It may then have the necessary quantity of supermolten gold to form the desired coating cast directly against it, access of air to the steel being of course avoided. Another convenient procedure is to raise the steel ingot from the heating furnace into a bottomless casing kept full of producer gas, or other non-oxidizing gas, transfer the casing over the bath of supermolten gold, lower the ingot into the bath a sufficient time—ordinarily a few seconds suffices—to cover the steel with a film of cohering gold, withdraw it into the casing, move the casing over an ingot mold, transfer the ingot to the mold and then cast about it, or in contact with it, sufficient gold at ordinary casting temperature, to form the desired thickness of coating. Or, after dipping the ingot into the supermolten gold, the casing may then be lowered around it, segregating a layer of the supermolten gold in immediate contact with the ingot, a bottom plate affixed and the casing then withdrawn carrying the ingot and the layer of gold.

Ordinarily the ingot should be heated, but not to the full supermolten temperature of the gold. Upon then contacting it with the supermolten gold while the superficial layers of the steel acquire the necessary temperature for the union, this temperature persists but momentarily, the heat soaking inward in the ingot. Where the supermolten gold is relied upon to form the full thickness of the coating, the temperature of the layer of gold is also quickly reduced by conduction outward through the mold walls. It is generally quite important that the two metals should not be long in contact at the supermolten temperature, thereby avoiding detriment to either by solution or corrosion of the other.

At the supermolten temperature the gold is, as stated, quite reactive, and it is therefore better not to prolong contact.

As to the nature of the stated activity at the supermolten temperature or as to the nature of the union which is formed, this is not definitely settled. It may be that the two metals superficially alloy, and certain phenomena seem to indicate this, forming a very thin intermediate alloy-film; said alloy being either a physical or chemical mixture. Or it may be that the gold simply perfectly and molecularly wets the surface of the steel, forming a union therewith which is in the nature of a molecular interpenetration or interlocking in which the molecules of the two metals cohere as the like molecules of each cohere to each other. But whatever the cause, the fact of a perfect union exists; a true cohesion as distinguished from a mere adhesion or sticking together. Where it is desired to work with the gold at a lower or ordinary casting temperature, the steel may be film coated by a dip into supermolten copper; or copper at a temperature of several hundred degrees above its melting point or ordinary casting temperature. With the coppered surface so prepared, in which the copper coheres to the steel, gold at an ordinary casting temperature may be now applied.

In the accompanying illustrations I have shown, more or less diagrammatically certain material and means adapted to perform the stated process.

In said drawings:—Figure 1 represents a sectional view of one form of apparatus for carrying out the said process. Fig. 2 shows in detail section the construction of bottom plate and lower portion of casing preferably employed. Fig. 3 shows a sectional view of another form of casing which may be employed.

In Fig. 1, 1 is a preliminary heating chamber for the ingot or core, 2 a furnace for heating a crucible 3, containing a body of supermolten coating metal, and 4 designates a second crucible, which may or may not be used, as desired.

5 designates a power hoist, here shown as an electrical hoist, mounted on a suitable track so that it can be moved from place to place; and from said hoist is suspended, by means of a porter bar 6, the ingot 7, which is the object to be coated. Said ingot is shown surrounded by a casing 8 having an internal diameter slightly larger than the external diameter of the ingot, and to said casing is connected a pipe 9, a portion of which is flexible, said pipe provided with a three-way valve 10. This pipe and the valve 10 are provided for supplying to the casing, when desired, an atmosphere of indifferent or neutral gas, such as producer gas. Casing 8 has a weighted head 11 which insures that when the casing is low-

ered into the molten metal it shall sink therein to the depth desired.

12 designates a bottom plate for the casing arranged to be secured to the ingot 7 itself, by means of a screw 13. Said bottom plate is provided with a raised rib or ring 14 matching a corresponding groove 15, in the lower edge of the casing, and adapted to coact with said groove to make a tight joint. 10 For raising and lowering the casing 8 with respect to the ingot 7, a special hoist 16, suspended like porter bar 6 from hoist 5, is provided. It has, in the form shown, two winding drums 17 upon which are wound two 15 cables 18 connected to opposite sides of the casing, so that said casing may be raised and lowered truly vertically.

I customarily provide the crucible with a loose removable cover 19, which cover is designed to exclude air from the molten metal 20 so far as possible, and is removed only when and so long as necessary to lower an ingot and casing into the crucible, or to inspect the molten metal, or for similar reason. To further exclude air from the surface of the molten metal, I cover so much of its surface as possible with a layer of charcoal, a ring 20 of refractory material which floats on the surface of the molten metal serving to maintain 30 a clear space in the center for the passage of the ingot and casing.

As an alternative to the above described apparatus for carrying out my process, I may use that shown in Fig. 3, which is much the same as that above described except that the casing 8 is provided with inlets 23 in its sides, said inlets arranged to be closed at will by a sliding shield or valve 24. In carrying out the process with this apparatus the casing 40 without the bottom plate 12 thereon is placed over the heating chamber 1, said casing being at the time filled with a protective atmosphere as above described, and the porter bar is lowered down through the casing, secured to the ingot or core to be coated and raised up into said casing again with the said 45 ingot or core. The casing with the core 7 within it, is then moved to one side, the bottom plate 12 applied, and then the casing is moved over the crucible 3 containing supermolten coating metal, and is lowered into 50 said supermolten metal; the valve or closure 24 being raised as the openings 23 come to the surface of the molten metal so that said 55 casing fills through said openings 23. The casing with ingot and molten metal within it is then raised and the molten metal allowed to cool as before. In carrying out the process in this way, the protective atmosphere 60 within the casing when the filling holes 23 are open, protects the surface of the ingot and the molten metal which enters the casing against oxidation; and in fact no air can enter the casing, because the holes 23 are submerged in the molten metal almost instantly 65

after the closure 24 is raised, and during the possible brief instant while said openings are open but not completely submerged the outrush of gas from the casing will prevent the entrance of air.

To hasten the filling of the casing with molten metal, and to prevent trapping of gas in the molten metal as it solidifies, I preferably apply suction to the outlet 25 of valve 10, having first set said valve so as to cut off the entrance of gas and to place outlet 25 in communication with the interior of the casing. This is done, however, only after the molten metal has commenced to flow in. And when necessary or expedient, I reduce the fluid pressure upon the joint between the bottom plate and casing, while raising either the casing shown in Fig. 1 or the casing shown in Fig. 3, by applying suction to the outlet 25 of valve 10.

The coated ingot produced in either of the ways above described is usually worked, as by rolling (either at once, or after submergence to a "soaking" heating to bring all the parts to a uniform temperature), to condense the metal of the coating and to extend it to shapes desirable for future working, such as bars, rods, and plates. In such extension the joined metals extend together without rupture of union and between them and the final article usually contains the same relative proportion of coating and base as the finished ingot.

The core or base or ingot coated as described in this specification need not be iron or steel, but for most purposes an iron or steel base or core will be preferred. Hence in certain of the following claims I specify steel as the metal of such core or base; and this term "steel" I employ generically to designate all forms of iron, including not merely ordinary carbon steel, both low-carbon or mild and high-carbon or hard, but also wrought iron (the properties of which are nearly identical with those of mild steel) and various compound steels, such as tungsten steel, titanium steel, vanadium steel, chrome steel, nickel steel, manganese steel, cobalt steel; also substantially pure iron—i. e., the chemical element Fe, substantially free from carbon and other metalloids or impurities and modifying ingredients.

In the methods of uniting gold and iron or steel above described, the excessively high temperature of the abutting layers of unlike metals exists only temporarily as the heat of the molten metal "soaks" into the steel core, while the heat of the molten metal is transferred outwardly by the cooling of the casing walls, and no opportunity is afforded for detrimental action upon either the main body of the steel or that of the molten metal. Such changes as take place, or may take place, in either metal, are only in the excessively thin joining layer between; and since, as already

explained, I do not limit myself to any theory of how the union between the unlike metals takes place, therefore I do not assert positively, that when the operation is properly 5 performed, any change of the two metals, or either of them, at the point of juncture, actually takes place. As previously explained, the time of contact of the steel and gold or other coating metal used, while such gold or 10 other coating metal remains in the supermolten condition, is very brief, for long contact of the two metals with the gold or other coating metal in the very high reactive condition afforded by the supermolten temperature, would of course be detrimental to 15 both. By limiting to a few seconds the period of contact of the metals while one of them is in the supermolten condition, I limit to extreme thinness the joining layer of alloyed, mixed, interpenetrating, or otherwise-united metals.

The steel coated in any of the foregoing ways possesses a cohering layer or stratum of gold which can be drawn, beaten or rolled 25 together with it at ordinary steel working temperatures without parting, even in the finest of wire, or in thin leaf. In an ingot so clad, a cutting tool, such as a cold chisel, refuses to discover or follow the line of union, 30 veering off into the softer metal; and heating and sudden quenching do not separate the joined metals.

Using very soft, pure iron, such as is obtained by the Tropenas process, or in blowing 35 melted iron till practically all carbon and metalloids are removed, for the ingot and coating with a comparatively thin layer of gold, a compound metal body is obtained which will stand extension into the thinnest 40 of gold leaf. Because of the opacity of the iron, the merest film of gold serves in the finished article. Such pure soft iron used as a core gives metal well adapted for jewelers use for making chains, rings, filled watch 45 cases and like purposes, after rolling or drawing down to the desired dimensions. When cut in the ordinary manner to form finished articles, the iron of course shows at exposed edges but by the use of certain 50 means and expedients, these cut edges may also have the core metal concealed. As set forth in my application filed March 2, 1906, Sr. No. 303,916, I have found that by cutting such compound metal, as for example a 55 plate of steel cored gold, with cutters or nippers with rounded or obtunded edges, giving a pinching cut, the core metal may be ruptured before the coating metal and the latter, so to speak, flowed down over its exposed edge.

60 Treatment with ordinary burnishing tools serves to complete the union of the metal so extended over the edge.

With a somewhat stiffer metal than the described soft iron, compound watch chains 65 may be made which are substantially safe

against rupture by pickpockets and thieves. Gold clad steel plates are eminently suitable for acid stills. The list of uses to which my new gold clad steel may be applied is of course practically endless, and those cited 70 are merely particular examples.

Instead of applying the coating in a single operation, as above described, I may apply it in two operations, film-coating the ingot 75 by immersing it momentarily in the supermolten metal in crucible 3 and then, without lowering the casing into the supermolten metal, withdrawing the ingot, now covered with a thin film-coating formed by the action of the supermolten metal, back into the casing, moving said casing over the crucible 4, the molten metal in which is preferably at ordinary casting temperature or thereabout, applying the bottom plate to the ingot, lowering said ingot into the metal of bath 4 and 80 thereafter lowering the casing and so confining against the film-coated surface a layer of the metal from bath 4, and then withdrawing the casing with its contents from the molten metal and permitting the molten metal with- 85 in it to solidify. Or, instead of using the apparatus of Fig. 1, that of Fig. 3 may be used; the consequent variation in the procedure 90 just described being obvious.

In case the operation is carried on in two 95 steps instead of one, the supermolten metal of bath 3 will ordinarily be some cheaper metal than gold which has the power of combining with iron or steel or other metal of which the base is composed, when in the supermolten condition, and with which the gold will combine at or near ordinary casting temperatures; copper for instance, though silver may be used. Employing a third metal in the supermolten bath is, in fact, 100 quite advantageous, for the reason that metals exposed to air or furnace gases or other contaminating influences while in the supermolten condition are very rapidly contaminated; which, if the supermolten metal be a precious metal, such as gold or silver, may add materially to the cost of the process, because of the waste of expensive metal involved. By employing a less expensive metal, such as copper, the possible loss due to contamination of the metal is greatly reduced. Gold at ordinary casting temperature will unite readily with a copper coating formed from supermolten copper, so as to be as inseparable from the copper as the copper is from the 110 iron or other base; and the thickness of the copper layer may be so slight as to be almost inappreciable, and quite inappreciable in the extended product.

I intend the term gold as used herein to 125 include such alloys or mixtures as are commonly termed "gold", even though the proportion of other metal be relatively great.

In application for Letters Patent filed April 17, 1907, Sr. No. 368,770, I have 130

claimed broadly a process of producing compound or clad metal articles comprising coating a surface of a metal base by contact with a supermolten mass of an unlike metal and then contacting the coating so formed with a molten mass of a third metal and causing a layer thereof to solidify thereon. In an application filed April 24, 1907, Sr. No. 369,997, I have claimed a process of forming compound or clad metal articles comprising contacting a surface of one metal with a supermolten mass of an unlike metal and confining a portion of the metal from such supermolten mass, of substantial thickness, in contact with such surface and causing it to solidify thereon. In an application filed June 19, 1908, Sr. No. 439,284, I have claimed compound or clad metal articles comprising a coating of copper, silver, gold, aluminum and like metals, alloyed with ferrous metals, weld-united to ferrous metals, and a process of making such articles. Therefore I do not claim such inventions in this case.

What I claim is:—

1. The process of making compound metal bodies which consists in contacting a ferrous metal base with a non-ferrous metal at a temperature much above its melting point and uniting a layer of a metal comprising gold to the treated base.

2. The process of making compound metal bodies which consists in contacting a ferrous metal base with a supermolten mass of non-ferrous metal, thereby forming on said base a coating, and uniting to said coating a layer of a metal comprising gold.

3. The process of making compound metal bodies which consists in uniting a ferrous metal and a metal comprising gold by contacting with the surface of said base a supermolten mass of a third metal, thereby forming on said base a coating, and uniting to said coating a layer of a metal comprising gold.

4. The process of making compound metal bodies which consists in uniting a ferrous

metal and a metal comprising gold by contacting with the surface of said base a supermolten mass of copper, thereby forming on said base a coating, and uniting to said coating a layer of a metal comprising gold. 50

5. The process of making compound metal bodies which consists in contacting a ferrous metal base with a non-ferrous metal maintained at a temperature much above its melting temperature and thereafter casting 55 molten gold against the treated base.

6. The process of making compound metal bodies which consists in contacting a ferrous metal base with copper maintained at a reactive temperature much above its melting 60 temperature and thereafter casting molten gold against the treated base.

7. The process of making compound metal bodies which consists in uniting a metal comprising gold and an unlike metal by contacting 65 a body of such unlike metal with a supermolten mass of a third metal and then casting molten gold-comprising metal against such body.

8. As a new article of manufacture, a compound metal body comprising a ferrous metal base and a poreless layer of a metal comprising gold united thereto by a union indisseverable by cutting tools or temperature changes. 70

9. As a new article of manufacture gold clad steel comprising a base of steel having a poreless layer of gold united thereto by an intermediate layer of a third metal of high melting point. 80

10. As a new article of manufacture gold clad steel comprising a base of steel having a poreless layer of gold united thereto by an intermediate layer of copper.

In testimony whereof I affix my signature, 85 in the presence of two witnesses.

JOHN F. MONNOT.

Witnesses:

J. F. KINDER,  
H. M. MARBLE.